

## UNITED STATES PATENT OFFICE

2,529,722

BUFFING AND POLISHING COMPOSITIONS  
AND METHOD OF PREPARATIONAllan E. Chester, Highland Park, Ill., assignor to  
Poor & Company, Chicago, Ill., a corporation of  
DelawareNo Drawing. Application August 27, 1948,  
Serial No. 46,563

10 Claims. (Cl. 51—305)

**1**  
This invention relates to buffing and polishing compositions and a method of preparation thereof.

In buffing and polishing brass, copper, nickel and other base metals, usually for finishing or preparatory to plating, two classes of abrasives have been employed, namely, natural abrasives such as carborundum, silica and quartz, and synthetic abrasives such as aluminum oxides, silicon carbides and precipitated ferric oxide, chromic oxide or other oxides. It is customary to employ binders such as waxes, tallow, stearic acid together with the abrasive in the buffing and polishing compositions. The buffing and polishing compositions are usually prepared in the form of a cake which can be applied to a buffing wheel and transferred to it prior to the polishing or buffing operation.

In preparing such buffing and polishing compositions, it has always been considered necessary heretofore to have the abrasive in an extremely fine, uniform particle size.

One of the objects of the present invention is to provide buffing and polishing compositions containing as an abrasive material a substance which has never been used before for this purpose and which is highly effective in such buffing and polishing operations.

Another object of the invention is to provide a new and improved buffing and polishing composition in which the active polishing agent exists in the composition in a relatively large range of particle sizes.

Still a further object of the invention is to provide a new and improved method for preparing buffing and polishing compositions. Other objects will appear hereinafter.

In accordance with the present invention it has been found that new and improved results are obtained in buffing and polishing operations by employing as the abrasive tailings from a conglomerate copper ore of the type found in Houghton, Keweenaw, and Ontonagon counties of northern Michigan, United States of America. The term "tailings" has a recognized meaning in the art pertaining to the recovery of copper from its ores and refers to the residue which is left after the ore has been treated to extract practically all of the copper, leaving iron and silicon as the principal constituents, together with alkali metals combined in the form of salts or complex oxides and smaller amounts of other metals.

In ordinary practice, the copper ore is mined, crushed, and extracted by procedures which in-

clude leaching, electrolysis, flotation and smelting. The ore is often treated, retreated and ground and the residue or tailings are finally discarded, usually by pumping them into a lake or a body of water. These tailings have found no large scale use up to the present time.

A typical analysis of such tailings taken from the conglomerate tailings of the Calumet & Hecla Company, near Calumet, Michigan, showed a hardness of 7.0 to 7.3 on the Moh scale. An analysis for size indicated the following:

|    | Retained on<br>Screen Mesh<br>(Openings per<br>Sq. In.) | Weight<br>Per Cent |
|----|---------------------------------------------------------|--------------------|
| 15 | 30                                                      | 5                  |
|    | 40                                                      | 7.5                |
|    | 60                                                      | 21.5               |
| 20 | 100                                                     | 34                 |
|    | 150                                                     | 8.5                |
|    | 200                                                     | 16                 |
|    | more than 200                                           | 7.5                |

These tailings contain about 4% moisture. A spectro-chemical analysis showed the presence of the following metals:

|                                   |                        |
|-----------------------------------|------------------------|
| Iron, Silicon                     | Principal Constituents |
| Potassium                         | 2 to 20%               |
| Sodium                            | 1 to 10%               |
| 30 Copper                         | 0.05 to 0.5%           |
| Chromium                          | 0.01 to 0.1%           |
| Aluminum                          | 0.01 to 0.1%           |
| Calcium                           | 0.01 to 0.1%           |
| Titanium                          | 0.001 to 0.01%         |
| 35 Vanadium                       | 0.001 to 0.01%         |
| Magnesium                         | 0.001 to 0.01%         |
| Tin, Silver, Nickel, Cobalt, Lead | traces <sup>1</sup>    |

<sup>1</sup> Less than 0.001% is present.

40 It is of interest to note that iron and silicon are the principal constituents and therefore the chief components of the substance which has been found to have unusual effectiveness as an abrasive in the practice of this invention. Heretofore it has been thought that iron could not be used in polishing chromium because it would cause discoloration. In the practice of the present invention, however, excellent results have been obtained in polishing chromium despite the presence of the iron.

45 A novel method is used in accordance with the present invention in order to incorporate the previously described tailings into a suitable buffing or polishing composition. This method is also applicable to the preparation of other types of

buffing and polishing compositions with other types of abrasives. The method may be described briefly as follows.

The conglomerated tailings in any suitable quantity, say in 40 pound to 100 pound batches, are wet milled with water, a gel-forming colloid, e. g., bentonite, and an electrolyte in order to make a slip or aqueous slurry similar in appearance to the slips or slurries which are made with vitreous enamel frits prior to applying and firing enamel. The slurry or slip is ground in a ball mill of the type used in grinding vitreous enamels until the particle sizes are reduced to at least  $\frac{1}{5}$  of the particle sizes in the tailings employed as the starting materials.

The preferred method of procedure is to ball mill the tailings with  $\frac{1}{4}\%$  to 3% by weight of bentonite,  $\frac{1}{4}\%$  to  $\frac{1}{4}\%$  by weight of sodium nitrite, magnesium sulfate or other electrolyte, and 35% to 45% water. This forms a colloidal slip which suspends the particles and facilitates further grinding in the ball mill. The amount of the grinding may be controlled depending upon the purpose for which the buffing composition is to be employed, for example, if the buffing composition is to be employed on die castings, the maximum particle size may be somewhat greater than in other applications, and the preferred maximum particle size in such case is 150 mesh. Where the buffing composition is to be employed for polishing aluminum, the preferred maximum particle size is 200 mesh. For a typical composition of the type just described 150 mesh maximum particle size can be obtained in about six hours, ball milling and 200 mesh maximum particle size can be obtained in about eight hours' ball milling. The product after ball milling has a multi-particle size similar to that of the original product but reduced by a ratio of around 5:1 to 8:1, depending upon the extent of the ball milling.

After the colloidal slip has been ball milled as previously described, it is run through a Roto-Spray to expel particles of any desired size, and it is then passed over a magnetic separator to remove any magnetic particles. After passing over the magnetic separator, it goes to settling tanks and is treated with agents which are known to cause separation of the water, such as, for example, tetrasodiumpyrophosphate and many other polyphosphates. These agents may be described as deflocculating and degelling agents. The excess water is removed by decantation and the resultant product is dried in the form of cakes. The cakes are broken up in a hammer mill and formulated into the final buffing composition. A typical final buffing composition may be prepared as follows:

| Parts by Weight | Ingredient                                                              |
|-----------------|-------------------------------------------------------------------------|
| 766             | Conglomerate tailings abrasive as prepared above.                       |
| 20              | Bentonite.                                                              |
| 50              | Stearic Acid (saponification #200-double saponified or triple pressed). |
| 30              | Hydrogenated fish oil (Hydrofol acids #51).                             |
| 100             | Crude scale wax.                                                        |
| 62              | No. 3292 petrolatum (Standard Oil of Indiana).                          |
| 20              | Hydrofol glycerides (M. P. 50-1° C.).                                   |

These ingredients melted together and molded form a suitable bar for buffing brass, aluminum, copper and other metals. The specified quantities in grams are sufficient to produce one bar.

In the foregoing composition the standard petrolatum No. 3292 has the following physical properties:

|                  |                 |
|------------------|-----------------|
| Specific gravity | 880-85          |
| Flash point      | 495° F.         |
| Fire point       | 555° F.         |
| Viscosity 210° F | 95-120 S. U. S. |
| Color            | 6-7             |
| Melting point    | 150-155° F.     |

Typical Hydrofol acids and glycerides which may be employed for the purpose of the invention have the following compositions:

|                                        | Hydrofol Glycerides 42 | Hydrofol Glycerides 50/51 | Hydrofol Acids 46 | Hydrofol Acids 51 |
|----------------------------------------|------------------------|---------------------------|-------------------|-------------------|
| 15 Melting point...°C.                 | 46.1                   | 55.8                      |                   |                   |
| Titre...°C.                            | 42.8                   | 52.4                      | 45.6              | 57.9              |
| Free fatty acid <sup>1</sup> per cent. | 0.9                    | 1.2                       | 100.7             | 100               |
| Iodine Value                           | 35.1                   | 3.9                       | 27.4              | 2.7               |
| Saponification Value                   | 190.2                  | 190                       | 200.1             |                   |
| Acid Number                            |                        |                           | 200               | 198.7             |

<sup>1</sup> Free fatty acid is oleic acid.

The crude scale wax has the following composition:

|                               |         |         |
|-------------------------------|---------|---------|
| 25 Melting point              | °F      | 122-132 |
| Viscosity (210° F.) (seconds) |         | 40-45   |
| Flash point (minimum)         | °F      | 400     |
| Oil content (maximum)         | percent | 20      |
| (minimum)                     | percent | .2      |

30 Weight (pounds per gallon)

The name "Hydrofol" is the trade name of the Werner G. Smith Company, Cleveland, Ohio, for hydrogenated fish oils and acids as described above.

35 From the foregoing illustration, it will be seen that the final abrasive composition is composed principally of the abrasive material and contains minor proportions of a gel-forming colloid and a binder. The binder in this case consists of the 40 stearic acid, hydrogenated fish oil, waxes and glycerides. The composition preferably contains about 70% to 75% of the abrasive material, about  $\frac{1}{4}\%$  to 1% of bentonite and the remainder a wax type binder.

45 It will be understood that abrasives prepared in the manner previously described may be incorporated with any buffing composition. Such compositions may contain as much as 75% of the abrasive and the remainder being a paraffin 50 wax, stearic acid or other type of amorphous binder. It is also desirable to incorporate with the buffing composition as much as  $\frac{1}{4}\%$  to 2% of a grease-soluble wetting agent, for example, the wetting agent sold under the name "Igepal".

55 The terms "buffing" and "polishing" are used herein in their conventional sense as employed in the art. "Polishing" usually refers to a roughing out process while "buffing" refers to the final finishing.

60 The compositions of the invention have been extremely effective in the buffing and polishing of various metals including chromium, aluminum and copper, even in the more difficult types of buffing, such as die cast buffing. The results obtained are surprising in view of the fact that the abrasive particles are of varying particle sizes, whereas the art has always attempted to reduce the abrasive particles to a uniform size. A further surprising result is the fact that the presence of iron in these particles does not mar or discolor chromium surfaces. The invention also provides a way of utilizing waste materials which heretofore have been of virtually no value and have presented a disposal problem. Another advantage of the invention is that the compositions

70

75

herein described can be employed for buffing stainless steel or chromium plate without using aluminum oxide or chromic oxide.

The invention is hereby claimed as follows:

1. A buffing and polishing composition comprising a mass of binder material and comminuted abrasive material distributed therethrough, said abrasive material consisting essentially of multi-sized particles derived by grinding tailings of conglomerated copper ore.

2. A buffing and polishing composition comprising a mass of binder material and comminuted abrasive material distributed therethrough, said abrasive material consisting essentially of multi-sized particles derived by grinding tailings of conglomerated copper ore having a Moh scale hardness of at least 7.0.

3. A buffing and polishing composition comprising a mass of binder material and comminuted abrasive material distributed therethrough, said abrasive material consisting essentially of multi-sized particles derived by grinding multi-sized abrasive particles of tailings of conglomerated copper ore of which at least 5% is retained on a 30 mesh screen and not more than 7.5% will pass through a 200 mesh screen until the particle size has been reduced 5 to 8 times.

4. A buffing and polishing composition comprising a mass of binder material and comminuted abrasive material distributed therethrough, said abrasive material consisting essentially of multi-sized particles derived by grinding multi-sized abrasive particles of which at least 5% is retained on a 30 mesh screen and not more than 7.5% will pass through a 200 mesh screen until the particle size has been reduced 5 to 8 times, said multi-sized particles consisting essentially of tailings from a conglomerate copper ore found in northern Michigan having a Moh scale hardness of at least 7.0 and comprising principally iron and silicon with smaller amounts of alkali metals and less than 0.5% of copper and other metals.

5. A buffing and polishing composition, comprising a mass of binder material and a gel-forming colloid and a comminuted abrasive material distributed therethrough, said abrasive material being derived by grinding tailings from conglomerate copper ore of the type found in northern Michigan.

6. The process of preparing an abrasive which

comprises milling a multi-particle sized abrasive with a gel-forming colloid, an electrolyte and water to form a colloidal slip, ball milling said slip until the desired particle sizes in said abrasive are obtained, separating magnetic particles from the resultant composition, then treating the resultant product with a deflocculating and degelling agent to cause separation of the water therefrom, drying the product into cakes, breaking up the cakes and incorporating the produce derived from the broken up cakes with a binder material.

7. A process as claimed in claim 6 in which the abrasive particles are subjected to ball milling until the maximum particle size is 150 mesh.

8. A process as claimed in claim 6 in which a gel-forming colloid is incorporated with the abrasive material and the binder.

9. A buffing and polishing composition comprising essentially a minor proportion of a waxy binder and a major proportion of multi-sized particles derived by grinding tailings from a conglomerate copper ore found in northern Michigan having a Moh scale hardness of at least 7.0 and comprising principally iron and silicon with smaller amounts of alkali metals and less than 0.5% of copper and other metals.

10. A buffing and polishing composition comprising essentially of 70% to 75% by weight of a comminuted abrasive material derived by grinding tailings from a conglomerate copper ore found in northern Michigan having a Moh scale hardness of at least 7.0 and comprising principally iron and silicon with smaller amounts of alkali metals and less than 0.5% of copper and other metals, and a wax-type binder.

ALLAN E. CHESTER.

#### REFERENCES CITED

40 The following references are of record in the file of this patent:

#### UNITED STATES PATENTS

| Number    | Name      | Date          |
|-----------|-----------|---------------|
| 45 92,962 | Hall      | July 27, 1869 |
| 2,078,876 | Hennessey | Apr. 27, 1937 |

#### FOREIGN PATENTS

| Number   | Country       | Date          |
|----------|---------------|---------------|
| 50 4,127 | Great Britain | of 1885       |
| 296,195  | Great Britain | Aug. 30, 1928 |